

F. W. GORDON.

## METAL REDUCING PROCESS.

APPLICATION FILED SEPT. 25, 1908. RENEWED SEPT. 9, 1910.

974,257

Patented Nov. 1, 1910.



Fig. 1.

WITNESSES:

Elmer R. Shipley.  
M. S. Beldin.



INVENTOR.

INVENTOR.  
BY James W. See  
ATTORNEY.

ATTORNEY.

# UNITED STATES PATENT OFFICE.

FREDERICK W. GORDON, OF PHILADELPHIA, PENNSYLVANIA.

## METAL-REDUCING PROCESS.

974,257.

Specification of Letters Patent.

Patented Nov. 1, 1910.

Application filed September 25, 1908, Serial No. 454,758. Renewed September 9, 1910. Serial No. 581,152.

To all whom it may concern:

Be it known that I, FREDERICK W. GORDON, a citizen of the United States, residing at Philadelphia, Philadelphia county, Pennsylvania, have invented certain new and useful Improvements in Metal-Reducing Processes, of which the following is a specification.

This invention pertains to improvements in processes for the reduction of the ores of volatile metals, and the improvements will be readily understood from the following description taken in connection with the accompanying drawing in which:

Figure 1 is a vertical diametrical section of a furnace exemplifying apparatus adapted for the carrying out of my improved process; Fig. 2 a horizontal section of the same; and Fig. 3 a vertical section of the cooler cut on a line concentric with the axis of the furnace.

The improved process may, perhaps, best be described by first describing the exemplifying apparatus.

In the drawing:—1, indicates the hearth of the furnace; 2, the general lower zone of the furnace; 3, the hopper; 4, the bell; 5, the downcomer; 6, the hot-blast tuyers; and 7, the tap-hole in the hearth.

All of the parts thus far referred to are, or may be substantially along the line of ordinary blast furnace construction, and subject to any of the usual or suitable modifications in such structures.

At this point it may be proper to consider the ordinary operation of the structure as thus far described, first, in the treatment of iron ores and, second, in the result of the operation when applied to the ores of volatile metals, regardless of whether the ores of the volatile metals be treated alone or be found in conjunction with the iron ores.

Assume the furnace to be working as usual with blast furnaces and dealing only with iron ores. In such case the usual re-actions will take place, the slag and iron being tapped from the hearth, and the resulting gases going to the downcomer. Assume, now, that instead of dealing wholly with iron ore, the ore is that of some volatile metal, say, zinc, and assume that line 8 indicates, in a general way, a point in the furnace-column of such high temperature as to vaporize reduced zinc, and assume that line 9 represents, in a general way, a point in the

furnace-column of such low temperature as to bring about the condensation of more or less of the zinc vapor developed at or below line 8. Under these conditions we would have zinc reduced and vaporized at line 8; we would have the zinc vapor driven upwardly to cooler regions in the furnace; we would have all or a portion of the zinc vapor condensed at line 9; we would have this condensed zinc descending again to the vaporizing regions of the furnace; we would have this descended zinc again vaporized and sent aloft; and this process might continue, the reduced zinc dancing vertically between the zones of vaporization and condensation. Not all of the zinc vapor would be condensed for some of it might be blown through the charge and to the downcomer, the ultimate result in any event being that there could be no recovery of zinc except such as could possibly be recovered from the gases blown out of the furnace. Thus far no reference has been had to additional charges to the furnace, but it is obvious that if no metallic zinc can pass below the level of vaporization no zinc can be recovered from the furnace as thus far described, except such as might be blown through the charge to the downcomer. By my improvements in process and apparatus I provide for withdrawing more or less of the gases from the furnace column at a point between the level of vaporization and the level of condensation, these gases carrying their quota of the zinc vapor. I recover a portion of the zinc by condensation in a cooler and I return to the furnace the withdrawn gases along with such zinc vapor as has not been condensed, the gases thus returned again entering upon their heating duty upon the charge, and the uncondensed zinc vapor going again to the furnace at a point above the level of vaporization.

Proceeding with the drawing:—8, and 9, indicate the two heat-levels heretofore referred to: 10, an annular cooler disposed around the furnace and divided by vertical walls into an annular series of chambers, eight being shown in the illustration, each of these chambers being, in turn, divided by up-standing and down-hanging walls into an odd number of vertical passes: 11, a port placing the interior of the furnace in communication with the foot of the first up-pass of each cooler chamber; 12, the first up-pass of a cooler-chamber; 13, the down-pass of a

cooler chamber: 14, the final up-pass of a cooler chamber: 15, a port placing the upper end of each final up-pass of the cooler in communication with the interior of the furnace: 16, a valve controlling each of the ports 15: 17, a zinc-tapping hole at the foot of each final up-pass of the cooler: 18, a sight-hole in the wall of the cooler over each of the zinc-tapping holes: 19, illuminating windows which it is desirable to provide at the foot of each final up-pass of the cooler to admit light at points opposite the sight-holes: 20, the middle zone of the furnace, which is the principal heating zone, this zone extending between the levels of ports 11 and ports 15: and 21, the upper zone of the furnace, above the ports 15, which zone may be considered the preliminary heating zone for the raw material of the charge.

20 Assume the furnace to be working, charged with fuel, zinc ore and fluxing material, and working at high temperature, say eighteen hundred deg. C. in the hearth, and assume that ores of iron or other non-volatile metal are present to some extent in the burden. So far as the ores of the non-volatile metals are concerned they will be reduced and go to the crucible and be tapped out with or below the slag, as in ordinary blast furnace practice, and as regards the zinc ores, they would be reduced only as heretofore described, the valves 16 being closed and no gases going to the cooler. Assume, now, that valves 16 be opened to a greater or less extent. The gases coming from the lower zone of the furnace, and comprising zinc vapor, will rise through the charge in the middle zone, as heretofore described. Much of the gas, seeking the path of least resistance, will leave the furnace column through the ports 11 and enter the cooler and rise therein and fall again and rise again and return to the furnace through the ports 15, the zinc vapors passing through the cooler having had their temperatures lowered so as to bring about partial condensation of the vapor and the deposit of metallic zinc at the feet of the final up-passes of the cooler, to be withdrawn at the zinc tapping-holes 17.

50 The gases leaving the cooler, including the uncondensed zinc vapor in them, return to the charge at the top of the middle zone and there mingle with the other gases in that zone, giving their heat to the charge and delivering their zinc vapor to the middle zone. The zinc vapor thus entering the middle zone becomes condensed to greater or less extent and works down to join with the zinc vapors forming in the lower zone. The gases then entering the cooler at ports 11 are the gases regularly formed in the lower zone of the furnace, except as modified by the descent among them of condensed zinc from the zinc vapor discharged into the furnace from the cooler. Therefore, assuming no additions to

the charge in the furnace, taking gases which have once passed through the cooler they return to the furnace and again to the cooler, and so on, becoming leaner and leaner at successive passages through the circuit, until finally substantially all of the zinc has been intercepted and tapped off. Assume, now, a working such as has been described, but with regular additional charges as usual in furnace practice. In such case the gases going to the cooler would never reach the condition of attenuation just spoken of, and the apparatus and its condition of working may be adjusted in such manner that the withdrawals of zinc from the cooler correspond with practical precision with the quantity represented by the zinc in the new charges.

The temperature at point of withdrawal of gases to the cooler are controlled by regulating the flow of gases through the cooler. This is effected by means of the valves in the outlets from the cooler which may be adjusted to determine what proportion of the total gases shall go through the cooler to have their heat dissipated. The greater the abstraction of gas to the cooler the more the temperature will be lowered at the entrance to the cooler, and the greater the abstraction the more this temperature will be increased.

It is to be understood that the upper zone 21 of the furnace is merely a convenient preliminary heating chamber to hold the supply of charge and to utilize the heat of the gases passing upward from the middle zone and from the cooler. So far as the principle of action of the apparatus is concerned, in its utilization of the gases discharged from the cooler, the supply of charge might be carried elsewhere, as in a bin, and be arranged to receive the gases coming from the cooler.

While the general construction and principle of operation has been above described it may not be out of place to here set forth more in detail the reactions taking place in the execution of the process.

The lower zone with its high hearth temperature, and fed with hot blast in judicious quantities, assures the formation of CO to the exclusion of CO<sub>2</sub>, the gases rising from the hearth being CO+N+ some H from the moisture of the blast. The lower zone is the region of carbon gasification by the blast, and reduction and vaporization of zinc. The temperature in the lower zone is sufficient to form and fuse ordinary blast furnace slag, and to reduce and fuse iron ore or other metallic ores non-volatile at its temperature. When the furnace with its cooler is regularly working on its burden of ore and flux and fuel, the burden in its descent meets the CO+N at higher and higher temperatures and becomes thereby heated, the ZnO parting with its O to form CO which rises with the gas; the ZnS of any combination being

split up, sulfur being volatilized and, rising with the  $\text{CO} + \text{N}$  encountering  $\text{CaO}$  and forming monosulfid.  $\text{CaS}$  descends and forms part of the slag.  $\text{ZnO}\text{CO}_2$  is split up by C to  $2\text{CO}$  and the  $\text{ZnO}$  gives its quota of O to the C, forming  $\text{CO}$ .  $\text{Zn}$  silicates are split, the silicates combining with lime forming part of the slag. Iron in any form is reduced to metal or rather pig metal and 10 may be tapped with or below the slag; this iron will assist in taking up sulfur if the lime is deficient. These reactions, for the most part, require high temperatures; these temperatures are met with successively during 15 the descent to the hearth, so that practically any ore may be split up and its constituents other than the vaporized metal acted on by the gases or the flux, giving zinc or other metallic vapor free from impurities. 20 The high hearth temperature is only limited by the blast temperature, economy of operation and durability of lining. Viewed in the light of blast, furnace practice, any required slag, even those with large lime and 25 alumina proportions, may be fused and tapped as a liquid. Upon the deoxidation of  $\text{ZnO}$ , or liberation of zinc from any of its compounds, it will be vaporized and diffused among the gases. A portion of this 30 mixture is caused to enter the cooler at a temperature approximating that of vaporization under the pressure within the furnace, assumed at 17 lbs. absolute or 2.3 lbs. gage per square inch, and leave the cooler at 35 a temperature about that of the solidification of zinc, avoiding fume formation in the cooler. If the density of the zinc vapor reaches its saturation point in the last up current in the cooler zinc globules will collect at 17; if not, this vapor being constantly formed will pass through openings 15 and thence through the cool charge in the upper zone, being solidified or oxidized. The 40 slowness of the current, fineness of the charge and considerable height of the column of charge will all tend to intercept the solid zinc, or zinc oxid, and carry it downward; meanwhile, the balance of the mixture will rise up the middle zone, some of its vapor 45 will condense, drop into a hotter region, re-vaporize, rise again with the gas and, dividing with the gas, a part of it will enter the cooler; the vapor thus entering the cooler, being denser by this addition, will pass 50 through the cooler, entering the furnace at 15 less that condensed in the cooler—and collect at 17. while the other portion of gas with this denser vapor will attempt an ascent of the middle zone. Part of the vapor first 55 rising through this shall have been solidified, caught in the charge and be coming back to be remelted and revaporized to join the vapor from condensed vapor and the vapor direct from reduced ore in further attempts to ascend among the charge and to 60 pass through the cooler. Thus the vapor, gradually made denser, is further supplied by the zinc caught in and returned from the upper zone, which has escaped condensation in the cooler; as all this vapor, new or from 65 zinc returned, is vaporized in and diffused in the lower zone, it rises with the gases generated in the hearth and acquires a density that will condense to liquid. The part of the gas carrying its proportion of vapor 70 passing through the cooler meets conditions for condensation and the collection of liquid zinc, and this is being constantly withdrawn from the aggregation of vapor diffused throughout the chambers. When this condition sets up in the cooler a condition is arrived at of continued condensation equal to the supply from the ore. 75

If the charge of ore and flux to a unit weight of fuel of known quality were arrived at to meet all heat requirements of the initial operation, such as reduction, volatilization or fusion of zinc, slag formation and fusing, sensible heat in the waste gases, radiation from the furnace, twyer water, decomposition of the moisture of the blast and radiation from the cooler, wherein a definite weight of gas + zinc vapor is cooled per minute of time, then all the heat requirements or, rather, the sum of them will remain constant and no extra heat, no extra fuel and no extra gas be generated. As 80 the process develops zinc vapor accumulates or condenses, for, the reevaporation of condensed zinc, reduction of zinc oxid in the 85 furnace or remelting frozen zinc entails no loss over that already gained by the condensation of hitherto vaporized zinc, oxidation of hitherto reduced zinc and freezing of 90 liquid zinc, provided the gain of heat is so 95 located that it can be appropriated to advantage. Now, all these heat developments take place well up in the charge; as developed this heat is given to the charge and by the charge is carried down to zones of heat 100 utilization; then with zinc vapor accumulating, while weight and volume of gas remain constant, the condition of saturation must be reached and, if condensation does not set in, be surpassed, and condensation enforced, whatever may be the effect of other 105 gases present in retarding condensation. 110

I claim:—

1. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction 120
2. The method of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction 125
3. The method of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction 130

- and gasification and metal vaporization, and an upper one of metal-vapor condensation; withdrawing from between said zones some of the furnace gases with their quota of metal-vapor; condensing a portion of the metal-vapor contained in said withdrawn gases; and recovering the metal resulting from said condensation, substantially as set forth.

2. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; condensing a portion of the metal-vapor contained in said withdrawn gases; recovering the metal resulting from said condensation; and utilizing said withdrawn gases for preheating the charge, substantially as set forth.

3. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; condensing a portion of the metal-vapor contained in said withdrawn gases; recovering the metal resulting from said condensation; conveying the uncondensed withdrawn metal-vapor back to the zone of metal-vapor condensation in the column; and utilizing said withdrawn gases for preheating the charge, substantially as set forth.

4. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; condensing a portion of the metal-vapor contained in said withdrawn gases;

5. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; condensing a portion of the metal-vapor contained in said withdrawn gases; recovering the metal resulting from said condensation; conveying the uncondensed metal-vapor to the said zone of metal-vapor condensation; utilizing said withdrawn gases for preheating the charge; and conveying the unwithdrawn gases with their quota of metal-vapor to the zone of metal-vapor condensation, substantially as set forth.

6. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; condensing a portion of the metal-vapor contained in said withdrawn gases;

- recovering the metal resulting from said condensation; conveying the remaining withdrawn metal-vapor to said zone of metal-vapor condensation; utilizing said withdrawn gases for preheating the charge; conveying the unwithdrawn gases with their quota of metal-vapor to the zone of metal-vapor condensation; returning to the zone of metal-vaporization the metal condensed in the zone of metal-vapor condensation from the withdrawn and unwithdrawn metal-vapor conveyed to it; enriching the withdrawn gases by adding thereto the metal-vapor returned from the zone of metal-vapor condensation; and continuing thus to enrich the withdrawing gases until the quantity of metal being recovered per unit of stock charged is approximately equal to the quantity of volatile metal contained in a unit of stock charged, substantially as set forth. 45
7. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; condensing a portion of the metal-vapor contained in said withdrawn gases; recovering the metal resulting from said condensation; conveying the remaining withdrawn metal-vapor to said zone of metal-vapor condensation; utilizing said withdrawn gases for preheating the charge; conveying the unwithdrawn gases with their quota of metal-vapor to the zone of metal-vapor condensation; returning to the zone of metal-vaporization the metal condensed in the zone of metal-vapor condensation from the withdrawn and unwithdrawn metal-vapor conveyed to it; enriching the withdrawn gases by adding thereto the metal-vapor returned from the zone of metal-vapor condensation; and continuing thus to enrich the withdrawing gases until the quantity of metal being recovered per unit of stock charged is approximately equal to the quantity of volatile metal contained in a unit of stock charged, substantially as set forth. 50
8. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; regulating the temperature at the point of such withdrawal by modifying the quantity of the withdrawn gases; condensing a portion of the metal-vapor contained in said withdrawn gases; and recovering the metal resulting from said condensation, substantially as set forth. 55
9. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; regulating the temperature at the point of such withdrawal by modifying the quantity of the withdrawn gases; condensing a portion of the metal-vapor contained in said withdrawn gases; and recovering the metal resulting from said condensation, substantially as set forth. 60
10. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; regulating the temperature at the point of such withdrawal by modifying the quantity of the withdrawn gases; condensing a portion of the metal-vapor contained in said withdrawn gases; and recovering the metal resulting from said condensation, substantially as set forth. 65
11. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; regulating the temperature at the point of such withdrawal by modifying the quantity of the withdrawn gases; condensing a portion of the metal-vapor contained in said withdrawn gases; and recovering the metal resulting from said condensation, substantially as set forth. 70
12. That improvement in the art of reducing the ores of volatile metals and recovering the metal therefrom which comprises the following steps, viz:—establishing and maintaining a columnar furnace-charge comprising commingled ore and fuel; establishing and maintaining therethrough an upward current represented by air injected at the base of the column and by gases discharged at the top of the column; establishing and maintaining within the column two successive zones, a lower one of reduction and gasification and metal-vaporization, and an upper one of metal-vapor condensation; withdrawing from between said zones some of the furnace gases with their quota of metal-vapor; regulating the temperature at the point of such withdrawal by modifying the quantity of the withdrawn gases; condensing a portion of the metal-vapor contained in said withdrawn gases; and recovering the metal resulting from said condensation, substantially as set forth. 75

FREDERICK W. GORDON.

Witnesses:

GEO. MECKE,  
WM. F. POTTER.